

[54] **PROCESS FOR SPINNING HIGH TENACITY FIBRES**

[75] Inventors: **Eric Frank Harris**, Greenisland, Northern Ireland; **John Francis Lloyd Roberts**, Harrogate, England

[73] Assignee: **Imperial Chemical Industries Limited**, London, England

[22] Filed: **Mar. 30, 1973**

[21] Appl. No.: **346,490**

[30] **Foreign Application Priority Data**

Apr. 6, 1972 Great Britain ..... 15848/72

[52] **U.S. Cl.** ..... **214/210 F**, 280/47 C, 264/290 T

[51] **Int. Cl.** ..... **D01f 3/10**

[58] **Field of Search** ..... 264/168, 290 T, 176 F, 264/210 F; 260/47 C

[56] **References Cited**

UNITED STATES PATENTS

3,361,859 1/1968 Cenzafo ..... 264/210 F

|           |         |                       |          |
|-----------|---------|-----------------------|----------|
| 3,624,031 | 11/1971 | Kobayashi et al. .... | 260/47 C |
| 3,642,697 | 2/1972  | Kobayashi et al. .... | 260/47 C |
| 3,654,225 | 4/1972  | Kobayashi et al. .... | 260/47 C |
| 3,689,623 | 9/1972  | Kobayashi et al. .... | 260/47 C |

FOREIGN PATENTS OR APPLICATIONS

|           |         |                     |           |
|-----------|---------|---------------------|-----------|
| 1,047,978 | 11/1966 | Great Britain ..... | 264/290 T |
| 44-2502   | 2/1969  | Japan .....         | 264/210 F |

*Primary Examiner*—Jay H. Woo

*Attorney, Agent, or Firm*—Roderick B. Macleod; Stephen D. Murphy; Thomas J. Morgan

[57]

**ABSTRACT**

Poly(ethylene-1:2-diphenoxylethane-4:4'-dicarboxylate) extruded to give spun yarn birefringence above  $60 \times 10^{-3}$  and not above value by equation  $\Delta = 18 \times 10^{-6} W + 50 \times 10^{-3}$  where  $\Delta$  is spun yarn birefringence and  $W$  is wind up speed, followed by orientation by extension.

**5 Claims, No Drawings**

## PROCESS FOR SPINNING HIGH TENACITY FIBRES

The present invention relates to the manufacture of yarns by the melt-spinning of poly(ethylene-1:2-diphenoxymethane-4:4-dicarboxylate).

According to the present invention we provide a process for the manufacture of a yarn of poly(ethylene-1:2-diphenoxymethane-4:4'-dicarboxylate) or its copolyester wherein poly(ethylene-1:2-diphenoxymethane-4:4'-dicarboxylate) or a copolyester of it is extruded under conditions to give a spun yarn of birefringence in excess of  $60 \times 10^{-3}$ , but not in excess of the value given by the equation

$$\Delta = 18 \times 10^{-6} W + 50 \times 10^{-3}$$

where  $\Delta$  is the spun yarn birefringence and  $W$  is the wind up speed, followed by orientation by extension.

Preferably the spun birefringence should be in excess of  $110 \times 10^{-3}$  and should not exceed the value given by the equation

$$\Delta = 16.2 \times 10^{-6} W + 50 \times 10^{-3}$$

By a copolyester of poly(ethylene-1:2-diphenoxymethane-4:4'-dicarboxylate) we mean a copolyester of which at least 90 percent of the structural units are of the formula:



Such copolymers may contain in the chain minor amounts of other structural units derived from glycols other than ethylene glycol and/or from dicarboxylic acids other than bis-1:2-(paracarboxyphenoxy)ethane and/or from a hydroxycarboxylic acid.

The poly(ethylene-1:2-diphenoxymethane-4:4'-dicarboxylate) or its copolyester for use in accordance with our invention may be manufactured by known methods and may contain one or more additives, for example delustrants, pigments, optical brighteners or stabilizers.

The yarns of our invention are of particular value when the poly(ethylene-1:2-diphenoxymethane-4:4'-dicarboxylate) or copolyester comprising them is of relative viscosity, as measured in orthochlorophenol at a concentration of 1 g. per 100 ml. of solvent and at a temperature of 25°C., greater than 2.0.

We have found it preferable to operate the process of our invention so that the spun yarn produced is amorphous, while still having a high spun birefringence. The preference for amorphous yarn arises from the fact that crystallinity in the spun yarn results in lower extensibility in the drawn product. By "amorphous" we mean that examination by X-ray diffraction showed no crystallinity.

The crystallinity of the spun yarn may be controlled by appropriate choice of relative viscosity of the poly(ethylene-1:2-diphenoxymethane-4:4'-dicarboxylate) and of the parameters of the melt-spinning. Thus crystallinity is favoured by increase in stress which is increased by increase in relative viscosity, increase in spinneret hole size for a given spun denier, reduction in the temperature of the poly(ethylene-1:2-diphenoxymethane-4:4'-dicarboxylate) at extrusion, increase in rate of

cooling in the molten region of the threadline, and increase in draw-down during spinning.

The ease of drawdown in forming the spun yarn will be inversely related to the viscosity of the extrudate, and the desirable spinning temperature will increase with yarn relative viscosity. We have found that for relative viscosities from 2.0 to 2.3 the desirable spinning temperature is in the range 295° to 335° C. In the case of the higher relative viscosities, it may be preferable to reduce the rate of filament cooling, for example by the use of a heated threadline shroud as described in U.K. Pat. No. 1,052,067, rather than to use impractically high extrusion temperatures.

Spun yarns of poly(ethylene-1:2-diphenoxymethane-4:4'-dicarboxylate) have the characteristic that when heated under low or zero tension they either shrink or increase in length spontaneously dependent on the initial spun yarn birefringence and on the temperature of heating. We have found that if we prefer to draw yarns of high birefringence, then there is less danger of undesirable spontaneous expansion prior to drawing if the value of the birefringence is at or above  $110 \times 10^{-3}$ . Below this value the spontaneous expansion of the product renders it more difficult to maintain control of spun yarn tension as it passes over heated surfaces.

When the spun yarn expands spontaneously under zero tension as described above it also crystallises, the crystalline form (referred to as  $\beta$  crystallinity) has a monoclinic habit.

The crystallisation which occurs under stress, as during spinning, is of a different crystalline form having an orthorhombic habit (referred to as the  $\alpha$  form). We have found that crystallisation under stress produces the  $\alpha$  form; thus the crystallisation obtained under the spinning stress and during drawing using a pin only, for example as described in our U.K. Specification No. 1,047,978, is of the  $\alpha$  form.

We have found, in our production of high relative viscosity high tenacity yarns that the modification of the drawing conditions to introduce some  $\beta$  crystallinity in the drawn yarn is beneficial, provided that the relative viscosity is above about 2.00.

When the cooling of the molten threadline is effected by contact with the ambient air at normal room temperature, the relationship between spun yarn relative viscosity and extrusion temperature to yield optimum tensile properties in the yarn after drawing is given by the equation:

$$\text{Extrusion temperature} = (89 \times \text{relative viscosity} + 128)^\circ \text{C.}$$

An advantage of the process of our invention is that by the use of it drawn yarns may be produced having a tenacity of greater than 9.5 g. per denier and an extension to break greater than 7 percent. Such yarns are of particular advantage for the manufacture of ropes, and cords. The cords are of particular use in the manufacture of tyres and V-belts, in which high modulus, good hydrolytic stability and low shrinkage are desirable. In the case of the use of the yarns in ropes, the good light stability is a further advantage.

The orientation by extension, that is drawing, may be carried out by known methods. Heated feed rolls or heated snubber pins may be used; we have found the latter to be preferable.

In order that our invention may be more clearly understood, we give hereinafter examples of methods in which it may be carried out.

## EXAMPLES 1 - 20

Poly(ethylene-1:2-diphenoxylethane-4:4'-dicarboxylate) of relative viscosity (R.V.), as measured in 1 percent by weight solution in orthochlorophenol at 25°C. as shown in Table 1 was melt-spun at a temperature as shown in Table 1. Other spinning conditions and the resultant spun birefringences are also given in Table 1.

TABLE 1

| Example | No. of Filaments | Spinneret hole diam. inches | Yarn RV. | Extrusion Temperature °C. | Shroud Temperature °C. | Wind Up Speed fpm.   | Spun Birefringence   | Yarn Morphology |
|---------|------------------|-----------------------------|----------|---------------------------|------------------------|----------------------|----------------------|-----------------|
| 1       | 3                | .035                        | 2.04     | 280                       | None                   | 500                  | $8 \times 10^{-3}$   | Amorphous       |
| 2       |                  |                             |          |                           | 1000                   | $21 \times 10^{-3}$  | do.                  |                 |
| 3       |                  |                             |          |                           | 1500                   | $58 \times 10^{-3}$  | do.                  |                 |
| 4       |                  |                             |          |                           | 2000                   | $88 \times 10^{-3}$  | $\alpha$ -form       |                 |
| 5       |                  |                             |          |                           | 2500                   | $98 \times 10^{-3}$  | do.                  |                 |
| 6       |                  |                             |          |                           | 3500                   | $115 \times 10^{-3}$ | do.                  |                 |
| 7       | 3                | .020                        | 2.00     | 301                       | 305                    | 1000                 | $3.2 \times 10^{-3}$ | Amorphous       |
| 8       |                  |                             |          |                           | 2000                   | $11 \times 10^{-3}$  | do.                  |                 |
| 9       |                  |                             |          |                           | 3000                   | $22 \times 10^{-3}$  | do.                  |                 |
| 10      |                  |                             |          |                           | 4000                   | $53 \times 10^{-3}$  | do.                  |                 |
| 11      |                  |                             |          |                           | 5000                   | $112 \times 10^{-3}$ | do.                  |                 |
| 12      |                  |                             |          |                           | 6000                   | $145 \times 10^{-3}$ | do.                  |                 |
| 13      | 3                | .009                        | 2.07     | 292                       | None                   | 4500                 | $132 \times 10^{-3}$ | $\alpha$ -form  |
| 14      | 3                | .009                        | 2.05     | 303                       | None                   | 4500                 | $118 \times 10^{-3}$ | Amorphous       |
| 15      | 48               | .015                        | 2.13     | 312                       | None                   | 4500                 | $133 \times 10^{-3}$ | $\alpha$ -form  |
| 16      | 48               | .015                        | 2.07     | 311                       | None                   | 4500                 | $125 \times 10^{-3}$ | Amorphous       |
| 17      | 3                | .020                        | 2.00     | 302                       | None                   | 4000                 | $139 \times 10^{-3}$ | $\alpha$ -form  |
| 18      | 3                | .020                        | 2.00     | 310                       | 305                    | 6000                 | $145 \times 10^{-3}$ | Amorphous       |
| 19      | 3                | .035                        | 1.96     | 290                       | None                   | 5000                 | $150 \times 10^{-3}$ | $\alpha$ -form  |
| 20      | 3                | .009                        | 1.96     | 290                       | None                   | 6000                 | $146 \times 10^{-3}$ | Amorphous       |

RV signifies relative viscosity.

fpm do. feet per minute.

Examples 1 - 10 are not according to the present invention.

## EXAMPLES 21 - 27

These Examples show that inferior drawn yarns are obtained from  $\alpha$ -crystalline spun yarn.

Yarns of 48 filaments having relative viscosities of 2.07 and 2.13 respectively were extruded at about 310°C. and wound up to give spun yarns of birefringence about  $130 \times 10^{-3}$ .

35 The following Examples show how in the absence of external heating effects, for example a threadline shroud, the spinning extrusion temperature varies with relative viscosity for the processes found to yield the best drawn tensile properties at a given relative viscosity level.

40 The results are shown in Table 3.

## EXAMPLES 28 - 33

TABLE 2

| Example | Yarn RV | Spun Yarn Morphology          | Spun Birefringence   | Max. Drawn Yarn Tenacity gm/denier | Single Filament Tenacity gm/denier | Tensile Properties Extension % | 2% Modulus gm/denier/100% Extension |
|---------|---------|-------------------------------|----------------------|------------------------------------|------------------------------------|--------------------------------|-------------------------------------|
| 21      | 2.07    | Amorphous                     | $125 \times 10^{-3}$ | 8.9                                | 9.8                                | 8.2                            | 198                                 |
| 22      |         |                               |                      | 8.4                                | 9.2                                | 8.5                            | 197                                 |
| 23      |         |                               |                      | 8.0                                | 8.8                                | 8.9                            | 194                                 |
| 24      |         |                               |                      | 7.1                                | 7.8                                | 11.0                           | 170                                 |
| 25      | 2.13    | Largely $\alpha$ -Crystalline | $133 \times 10^{-3}$ | 8.7                                | 9.6                                | 6.6                            | 219                                 |
| 26      |         |                               |                      | 8.0                                | 8.8                                | 7.5                            | 184                                 |
| 27      |         |                               |                      | 7.2                                | 7.9                                | 9.1                            | 158                                 |

TABLE 3

| Example | RV in O.C.P. | Spun Birefringence   | Extrusion Temperature °C. | Maximum Yarn Tensile Properties     | No. of filaments |     |
|---------|--------------|----------------------|---------------------------|-------------------------------------|------------------|-----|
|         |              |                      |                           | 2% Modulus gm/denier/100% Extension |                  |     |
| 28      | 1.53         | $5.5 \times 10^{-3}$ | 265°                      | 5.4                                 | 3.8              | 174 |
| 29      | 1.79         | $106 \times 10^{-3}$ | 290°                      | 9.3                                 | 4.6              | 220 |
| 30      | 1.84         | $99 \times 10^{-3}$  | 290°                      | 9.5                                 | 6.3              | 203 |
| 31      | 2.02         | $130 \times 10^{-3}$ | 312°                      | 9.6                                 | 7.1              | 197 |
| 32      | 2.08         | $95 \times 10^{-3}$  | 312°                      | 9.2                                 | 7.7              | 183 |
| 33      | 2.32         | $133 \times 10^{-3}$ | 330°                      | 9.4                                 | 7.0              | 183 |

## Example 28 is not according to the present invention.

From the data in Table 3 a trend line of optimum spinning temperature against yarn RV can be constructed. This relationship proves to be a good straight line curve which obeys the equation:

$$\text{Optimum Spinning Temperature} = 89 \times \text{RV} \text{ in } 1\% \text{ O.C.P} + 128^\circ \text{C.}$$

## EXAMPLE 34

This example shows how the dimensional stability of amorphous spun yarn varies as a function of spun birefringence and temperature of heat treatment.

Yarns having spun birefringences varying from  $4 \times 10^{-3}$  to  $173 \times 10^{-3}$  were spun. Hanks of these yarns were then suspended in a steam bath at  $100^\circ \text{C}$  for 15 mins. and their change in length measured. Further samples of the yarns were then suspended in an air oven at  $160^\circ \text{C}$  for 15 minutes and their change in length again measured. The data for the variation of change in length with initial spun yarn birefringence at  $100^\circ \text{C}$  and  $160^\circ \text{C}$  are given in table 7. From these data

## EXAMPLES 35 - 37

These examples demonstrate how both pin and plate temperatures affect the relative amounts of  $\alpha$  and  $\beta$ -crystalline forms in the drawn product.

5 A 24 filament yarn was spun in a similar manner to that in case II to an RV of 2.08 at  $312^\circ \text{C}$  and collected at 3,500 fpm to give an amorphous spun yarn of birefringence  $74 \times 10^{-3}$ . The yarn was shown to be capable of drawing at optimum conditions to give a product

10 having a filament tenacity in excess of 10.0 gm/denier.

The spun yarn was drawn at a fixed draw ratio of 2.9:1 over ranges of pin and plate temperatures and the relative proportions of  $\alpha$  and  $\beta$ -crystalline form in the product measured by x-ray diffraction techniques. The results are given in table 8. They indicate that the pin temperature fixes a limit on the level of  $\beta$ -form achievable, this limit decreasing with increased pin temperature. The furthermore show that the ease of attainment 15 of this limit rises rapidly with plate temperature above 170°C.

20 The results are shown in Table 5.

TABLE 5

| Example | Plate Temperatures | Relative percentage of monoclinic $\beta$ -form in the crystalline regions of the drawn yarn |       |       |       |
|---------|--------------------|----------------------------------------------------------------------------------------------|-------|-------|-------|
|         |                    | 150°C                                                                                        | 170°C | 190°C | 210°C |
| 35      | Pin Temperatures   | 100°C                                                                                        | 0     | 9     | 45    |
| 36      | do.                | 125°C                                                                                        | 7     | 11    | 30    |
| 37      | do.                | 150°C                                                                                        | 4     | 11    | 18    |
|         |                    |                                                                                              |       |       | 22    |

it can be seen that below a birefringence of about  $110 \times 10^{-3}$  the yarn shows a marked tendency to expand spontaneously. We have found that in the starting up of drawing processes which do not permit slip on the heated drawing surface the spontaneous expansion led to considerable difficulties which were significantly reduced at values above  $110 \times 10^{-3}$ . The results are shown in Table 4.

At  $100^\circ \text{C}$ . the change in length was determined by measurement of length of loops.

At  $160^\circ \text{C}$ . the change in length was calculated from the change in yarn denier.

## EXAMPLES 38 - 43

35 These examples show that if the yarn is drawn in such a way that the drawn product is predominantly crystalline in the  $\alpha$ -form the tensile properties are inferior, i.e., within a given context an increased proportion of  $\beta$ -form is favourable to tensile properties.

40 Filaments of relative viscosity 2.07 were extruded through a 48 hole spinneret at  $312^\circ \text{C}$  and wound up at speeds of 2,000 and 4,500 fpm to give spun yarns of birefringences 17 and  $125 \times 10^{-3}$ . The yarns were shown to be amorphous as spun.

TABLE 4

Variation of amorphous spun yarn dimensional stability at  $100^\circ \text{C}$ . and  $160^\circ \text{C}$ .

| Spun Birefringence   | 100°C              |                      | 160°C              |                    |
|----------------------|--------------------|----------------------|--------------------|--------------------|
|                      | % Change in length | Spun Birefringence   | % Change in length | Spun Birefringence |
| $3.4 \times 10^{-3}$ | -1.0               | $3.9 \times 10^{-3}$ | +6                 |                    |
| 3.9 do.              | -1.6               | 6.0 do.              | +4                 |                    |
| 6.0 do.              | -1.6               | 7.6 do.              | +11                |                    |
| 7.6 do.              | -1.4               | 11.8 do.             | +24                |                    |
| 10.4 do.             | +0.5               | 13.0 do.             | +14.2              |                    |
| 13.0 do.             | +4.2               | 27.0 do.             | +29                |                    |
| 13.9 do.             | +6.8               | 32.0 do.             | +26                |                    |
| 24.0 do.             | +16.3              | 46.0 do.             | +23                |                    |
| 27.0 do.             | +19.6              | 60.0 do.             | +18                |                    |
| 32.0 do.             | +19.2              | 69.0 do.             | +15                |                    |
| 38.0 do.             | +19.0              | 112.0 do.            | +5                 |                    |
| 46.0 do.             | +16.8              | 121.0 do.            | +4                 |                    |
| 61.0 do.             | +12.5              | 136.0 do.            | +3                 |                    |
| 68.0 do.             | +12.6              |                      |                    |                    |
| 81.0 do.             | +9.2               |                      |                    |                    |
| 95.0 do.             | +5.4               |                      |                    |                    |
| 113.0 do.            | +2.1               |                      |                    |                    |
| 125.0 do.            | +0.7               |                      |                    |                    |
| 135.0 do.            | +0.3               |                      |                    |                    |
| 160.0 do.            | -1.5               |                      |                    |                    |

The minus sign indicates that shrinkage occurs.

The plus sign indicates that elongation occurs.

The yarns were drawn over a heated pin and plate at a speed of 350 fpm, at the appropriate maximum draw ratio using the fixed optimum plate temperature while the pin temperature was varied. Data for these studies are given in table 6, the results show that above a pin temperature of 125°C a deterioration in extensibility occurs.

The results are shown in Table 6.

then fall off above a certain temperature.

At RV 2.08 the falling off in tenacity is evident at 205°C, but at RV 2.32 there is no change until 215°C is reached. Thus the optimum plate temperature rises with RV up to at least RV 2.32.

What we claim is:

1. A process for the manufacture of a yarn of poly (ethylene-1:2-diphenoxoethane-4:4'-dicarboxylate) or of

TABLE 6

| Example | Spun Birefringence   | Draw Ratio | Pin Temp. °C | Plate Temp. °C | Filament Tenacity gm/denier | Tensile Properties % Extension | 2% Modulus gm/den./100% Extn. | Crystalline Regions % β-form |
|---------|----------------------|------------|--------------|----------------|-----------------------------|--------------------------------|-------------------------------|------------------------------|
| 38      | $17 \times 10^{-3}$  | 5.8        | 105          | 196            | 8.8                         | 7.7                            | 194                           | —                            |
| 39      |                      | 5.8        | 125          | 196            | 9.2                         | 7.5                            | 200                           | 8                            |
| 40      |                      | 5.8        | 150          | 196            | 8.9                         | 6.3                            | 196                           | —                            |
| 41      | $125 \times 10^{-3}$ | 3.2        | 105          | 196            | 9.8                         | 8.2                            | 200                           | —                            |
| 42      |                      | 3.2        | 125          | 196            | 9.8                         | 7.9                            | 203                           | —                            |
| 43      |                      | 3.2        | 150          | 196            | 9.5                         | 6.8                            | 205                           | 13                           |

Examples 38, 39 and 40 are not according to the present invention.

#### EXAMPLES 44 - 52

Spun yarns were produced in a similar manner to that for Examples 38 - 43.

- A 24 filament yarn of RV 2.08 was extruded at 312°C and collected at 3,500 fpm to give a spun yarn which was amorphous and had a birefringence of  $74 \times 10^{-3}$ .
- A 24 filament yarn of RV 2.32 was extruded at 325°C and collected at 2,150 fpm to give a spun yarn which was partly α-crystalline and had a birefringence of  $92 \times 10^{-3}$ .

The two spun yarns were drawn at 350 fpm and a heated pin and plate to the appropriate maximum draw ratio using a fixed pin temperature while the plate temperature was varied. The effects of plate temperature on the tensile properties and on the percentage of β-crystalline form in the crystalline regions of the drawn yarns are shown in Table 7.

The results are shown in Table 7.

its copolyester in which at least 90 percent of the structural units are of the formula



said yarn having a tenacity in excess of 8.5 g.p.d. wherein poly (ethylene-1:2-diphenoxoethane-4:4'-dicarboxylate) or a copolyester of it having a relative viscosity greater than 2.0 is extruded under conditions giving a spun yarn of birefringence in excess of  $60 \times 10^{-3}$ , but not in excess of the value given by the equation:

$$\Delta = (18 \times 10^{-6}) W + (50 \times 10^{-3})$$

wherein Δ is the spun yarn birefringence and W is the wind-up speed in feet per minute, and W has a range of 500 to 6,000, followed by orientation by hot drawing at a draw ratio substantially defined by the value of 4.0 at a birefringence of  $74 \times 10^{-3}$ , 3.5 at a birefringence of  $92 \times 10^{-3}$ , and 3.2 at a birefringence of  $125 \times 10^{-3}$

TABLE 7

| Example | Spun Birefringence  | Yarn RV | Extrusion Temperature °C | Draw Ratio | Pin °C | Plate °C | Drawn β-Form % | Filament Tenacity gm/denier | Tensile Properties % Extension | 2% Modulus gm/den./100% Extn. | 100°C Shrinkage % |
|---------|---------------------|---------|--------------------------|------------|--------|----------|----------------|-----------------------------|--------------------------------|-------------------------------|-------------------|
| 44      | $74 \times 10^{-3}$ | 2.08    | 312°                     | 4.0        | 115    | 175      | 2              | 8.5                         | 6.0                            | 188                           | 4.2               |
| 45      |                     |         |                          | 4.0        | 120    | 188      | 12             | 10.1                        | 7.0                            | 230                           | 2.7               |
| 46      |                     |         |                          | 4.0        | 115    | 198      | 22             | 9.9                         | 7.3                            | 222                           | 2.5               |
| 47      |                     |         |                          | 4.0        | 120    | 205      | 18             | 9.6                         | 7.3                            | 225                           | 2.6               |
| 48      |                     |         |                          | 4.0        | 115    | 212      | 29             | 8.1                         | 7.6                            | 216                           | 2.2               |
| 49      | $92 \times 10^{-3}$ | 2.32    | 325°                     | 3.5        | 125    | 176      | 4              | 8.4                         | 6.4                            | 173                           | 4.0               |
| 50      |                     |         |                          | 3.5        | 125    | 196      | 7              | 8.9                         | 7.9                            | 170                           | 4.0               |
| 51      |                     |         |                          | 3.5        | 125    | 208      | 12             | 9.7                         | 8.0                            | 194                           | 4.0               |
| 52      |                     |         |                          | 3.5        | 125    | 215      | 13             | 9.0                         | 8.2                            | 177                           | 3.8               |

At both levels of RV the proportion of β-form increases with plate temperature whilst the tensile properties improve with increased plate temperature and

at conventional temperatures.

2. A process for the manufacture of a yarn according to claim 1 wherein the spun yarn birefringence is in ex-

cess of  $110 \times 10^{-3}$  but does not exceed the value given by the equation:

$$\Delta = (16.2 \times 10^{-6}) W + (50 \times 10^{-3}).$$

3. A process for the manufacture of a yarn according to claim 1 wherein said spun yarn is amorphous as judged by x-ray diffraction.

4. A process for the manufacture of a yarn according to claim 10 wherein the relative viscosity of the poly(ethylene-1:2-diphenoxymethane-4:4'-dicarboxylate) or 10 copolyester is up to 2.3 and the extrusion temperature

is in the range from 295° to 335° C.

5. A process for the manufacture of a yarn according to claim 1 wherein cooling of the molten threadline is effected by contact with the ambient air at normal temperature and the relationship between spun yarn relative viscosity and extrusion temperature is according to the following formula:

$$\text{Extrusion temperature} = (89 \times \text{relative viscosity} + 128)^\circ \text{C.}$$

\* \* \* \* \*

15

20

25

30

35

40

45

50

55

60

65